

# UNITED STATES PATENT OFFICE.

GEORGE ALBERT CHAPMAN AND STANLEY TUCKER, OF LONDON, ENGLAND, ASSIGNORS  
TO MINERALS SEPARATION LIMITED, OF LONDON, ENGLAND.

## ORE CONCENTRATION.

1,079,107.

Specification of Letters Patent. Patented Nov. 18, 1913.

No Drawing.

Application filed July 30, 1912. Serial No. 712,309.

*To all whom it may concern:*

Be it known that we, GEORGE ALBERT CHAPMAN and STANLEY TUCKER, subjects of the King of England, and both residing at 5 London, England, have invented certain new and useful Improvements in Ore Concentration, of which the following is a specification.

This invention is for improvements in or 10 relating to ore concentration.

A number of processes are known in which crushed ore is mixed with water containing a selective agent such as oil, or a mineral-frothing agent, and containing also 15 an acid such as sulfuric acid after which the metalliferous constituents of the ore are separated by flotation or the like. Such processes will hereinafter be referred to as flotation processes. Typical examples are 20 described in the previous Patents Nos. 835,120 of November 6, 1906, 879,985, of February 25, 1908, and 962,678, of June 28, 1910.

In some cases and for various reasons it is 25 disadvantageous to use an acid such as sulfuric acid. Thus the acid may not be readily obtainable or may be expensive or, for example with ores containing carbonates such as calcite, the acid may be rapidly con- 30 sumed.

It has been proposed in a flotation process as for example as described in United States Patent No. 835,120 mentioned above, wherein acid is used, not for its chemical action, 35 but for its physical effect, to use in place of the acid an acid salt, and also it has been proposed, in processes wherein acid is used for its chemical action, to treat an ore by introducing it into a hot solution containing 40 sulfuric acid or salt cake or a bisulfate of an alkali metal for the purpose of effecting the flotation of the sulfids by gas chemically generated by the acid without the employment of any selective agent or any mineral 45 frothing agent.

According to this invention, a process for the concentration of metalliferous ores consists in agitating the ore with water containing a selective agent or a mineral frothing 50 agent and containing also a bisulfate of an alkali metal or a mixture of a normal sulfate of an alkali metal and sulfuric acid; separating the metalliferous matter by flotation, and thereafter treating the liquor with

free acid to bring it back to its original condition and using it with or without a further quantity of the selective agent or mineral frothing agent for the treatment of a further quantity of ore. Also, according to 55 this invention, an ore containing a carbonate decomposable by sulfuric acid may be treated by subjecting it to agitation and to the action of a selective agent or a mineral frothing agent in the presence of a bisulfate of an alkali metal or of a normal sulfate of 60 an alkali metal and sulfuric acid.

When the acid generally employed is replaced by a bisulfate of an alkali metal, it is found that with a closed circuit, that is to say, using the same circuit liquor repeatedly, 70 the super-normal acid radical is slowly consumed, leaving normal sulfate. The sulfuric acid ( $H_2SO_4$ ) in light combination with normal sulfate ( $Na_2SO_4$ ) in the bisulfate ( $NaHSO_4$ ) will throughout the specification 75 be referred to as the available sulfuric acid. In the course of the process the available sulfuric acid is consumed if the ore contains carbonates or the like, but is consumed comparatively slowly and not until the acid has 80 had time to effect its desired physical action. To bring the liquor back into the desired condition, we add free sulfuric acid and lightly agitate to get the same effect as a solution of bisulfate of soda. In each case 85 the effect is to retard the consumption of the sulfuric acid, no doubt owing to what is known as the "balanced action".

The degree of advantage in using bisulfate instead of sulfuric acid, varies in different circumstances. For example, in using essential oils as frothing agents, the advantages of bisulfate over acid are not so marked as with other frothing agents, and indeed, with essential oils, acid can frequently be omitted with advantage, as mentioned for example in British Patent No. 21,857 of 1910.

The process of concentrating ores according to this invention is more particularly applicable to the concentration of a calcite blonde ore, that is, an ore containing carbonates. In one case we have investigated of a calcite blonde ore, the ordinary process of concentrating the ore by the flotation 105 method is to agitate it, after crushing, in four times its weight of water at about 60° C. with about one and one-half lbs.

per ton (0.067%) of an oily frothing agent. About 120 lbs. of acid per ton of ore (5.3%) must be added to insure a clean flotation and this is disadvantageous because of the high acid consumption and because sulfuric acid suddenly and rapidly attacks the carbonates, interfering with good concentration.

The following is a description by way of example of one method of carrying this invention into effect. The ore, a zinc-lead ore, to be treated, is mixed with water containing preferably about 1% of commercial bisulfate of soda (*i. e.* the  $H_2SO_4$  radical beyond the  $Na_2SO_4$  is equivalent to 36 lbs. of  $H_2SO_4$  per ton of ore, or 1.6%), and 1½ lbs. per ton of ore (0.067%) of wood tar oil and Texas fuel oil mixed in equal volumes. The mixture is agitated for about one-half minute at 55° C. and discharged into a spitzkasten where the froth which floats is removed with a certain quantity of water. The tailings from the spitzkasten are drawn into a second mixing vessel, agitated with a further quantity of wood tar oil and Texas fuel oil, and discharged into a second spitzkasten where a second froth is removed. The tailings are retreated in a third mixing vessel and so on, the operation being preferably carried out in the apparatus described in the prior Patent No. 979,857, of December 27, 1910. The liquid, passing off from the spitzkasten with the froth, is separated from the solid particles contained therein and is returned to the circuit for the treatment of a further quantity of ore. In many cases the bisulfate of soda used is equivalent to the use of 36 lbs. per ton of ore (1.6%) of available sulfuric acid and the consumption is less than this. When the liquid is returned to the circuit, sufficient sulfuric acid is added thereto to bring the quantity of available sulfuric acid back to the 36 lbs. per ton present in the original amount of bisulfate employed.

In the ordinary process of concentrating ores by froth flotation, a much larger percentage of acid would be necessary to insure a clean flotation than the 1.6% mentioned above, in some cases being as much as 10%.

The following is a description by way of example of another method of carrying this invention into effect: 400 grms. of a sample of San Francisco del Oro was agitated with 1600 c. c's of water containing 1% of bisulfate of soda, the equivalent of 36 lbs. per ton of available sulfuric acid and 1 lb. of camphor oil together with 1 lb. of wood tar oil per ton of ore, the temperature being that of the atmosphere. The recovery of zinc contents in two treatments was 77.6% and of the lead contents, 52.1%, the concentrates assaying zinc, 39.7% lead 14.8%, insolubles 2.9%, a very clean concentrate.

The following is a description by way of example of one method of carrying the in-

vention into effect when normal sodium sulfate and sulfuric acid are employed. The ore contained argentiferous galena (about 13%) blonde (about 30%) associated with quartz and fluor-spar. In 1600 c. c. of water were dissolved 21.5 grs. of Glauber salt  $Na_2SO_4 \cdot 10H_2O$  and 6.5 grs.  $H_2SO_4$ . This mixture was a agitated at 60° C. to effect uniform solution. 400 grs. of ore were added immediately followed by 0.04% of camphor oil (equivalent to one pound per ton of ore) and 0.007% amyłacetate (equivalent to 0.16 lbs. per ton of ore). This mixture was agitated for one minute and one froth removed gave a recovery of 85.7% of the zinc content and 57.3% of the lead content; an assay of the concentrate showed 37.3% of zinc, 13.9% of lead and 3.6% of insolubles. It will be seen that in this test the amount of available sulfuric acid used was about 1.6% on the ore, and the consumption was less than this whereas in using sulfuric acid in the ordinary way more than 10% of sulfuric acid is necessary to insure any clean flotation, because sulfuric acid by itself suddenly and rapidly attacks the carbonates.

An example of this invention as applied to film flotation, will now be described: 400 grms. San Francisco del Oro ore crushed to 60 mesh, was agitated with 1600 c. c. of water at atmospheric temperature containing Glauber salt and sulfuric acid equivalent to 1% of bisulfate of soda, and 5 lbs. per ton of Texas fuel oil, for one minute. The resultant pulp was floated at atmospheric temperature.

In carrying this invention into practice part of the metalliferous constituents may be separated by the process described in the previous Patent No. 879,985, hereinbefore mentioned.

It is found that the sodium bisulfate has the same physical effects as the sulfuric acid commonly employed in such processes, that is to say, it enables a sufficient recovery to be made but no rapid consumption of the reagent is noticeable and the same circuit liquor can be repeatedly used. Potassium bisulfate has the same effect as sodium bisulfate.

In the processes above referred to the details of practical operation may be varied. Thus the pulp may be at atmospheric temperature or may be heated to any suitable degree according to the conditions. The nature of the frothing agent and the stage or stages at which it is added may be varied. Either the concentrates or the tailings may be retreated with or or without the addition of further quantities of agents.

In carrying this invention into effect it is to be understood that the bisulfate may be formed or equivalent effects obtained by adding normal sulfate and sulfuric acid to the ore pulp.

What we claim as our invention and desire to secure by Letters Patent is:—

1. A process for concentrating ores, which consists in subjecting to agitation and to the action of a selective agent a pulp of an ore containing a carbonate, in the presence of a bisulfate of an alkali metal, and separating the selected portion of the ore.
2. A process for concentrating ores, which consists in subjecting to agitation and to the action of a selective agent a pulp of an ore containing a carbonate, in the presence of a sulfate of an alkali metal and sulfuric acid, and separating the selected portion of the ore.
3. A process for concentrating ores, which consists in subjecting an ore pulp to agitation and to the action of a selective agent, in the presence of a bisulfate of an alkali metal, separating the selected portion of the ore and solid residue from the liquor, and returning the liquor in closed circuit with the addition of sulfuric acid for the treatment of a further quantity of ore.
4. A process for concentrating ores, which consists in subjecting an ore pulp to agitation and to the action of a selective agent, in the presence of a sulfate of an alkali metal and sulfuric acid, separating the selected portion of the ore and solid residue from the liquor, and returning the liquor in closed circuit with the addition of sulfuric acid for the treatment of a further quantity of ore.
5. A process for concentrating ores, which consists in subjecting to agitation and to the action of a selective agent the pulp of an ore containing a carbonate, in the presence of a bisulfate of an alkali metal, separating the selected portion of the ore and solid residue from the liquor, and returning the liquor in closed circuit with the addition of sulfuric acid for the treatment of a further quantity of ore.
6. A process for concentrating ores, which consists in subjecting to agitation and to the action of a selective agent a pulp of an ore containing a carbonate, in the presence of a sulfate of an alkali metal and sulfuric

acid, separating the selected portion of the ore and solid residue from the liquor, and returning the liquor in closed circuit with the addition of sulfuric acid for the treatment of a further quantity of ore.

7. A process for concentrating ores, which consists in agitating a pulp of an ore containing a carbonate to beat in air and form a mineral froth in the presence of small proportions of a bisulfate of an alkali metal and a mineral frothing agent, and separating the froth produced.

8. A process for concentrating ores, which consists in agitating a pulp of an ore containing a carbonate to beat in air and form a mineral froth in the presence of small proportions of a sulfate of an alkali metal and sulfuric acid and a mineral frothing agent, and separating the froth produced.

9. A process for concentrating ores, which consists in agitating an ore pulp to beat in air and form a mineral froth in the presence of a small proportion of a bisulfate of an alkali metal and a mineral frothing agent, separating the froth produced, treating the liquor with free sulfuric acid, and using it with the addition of a further quantity of the mineral frothing agent for the treatment of a further quantity of ore.

10. A process for concentrating ores, which consists in agitating an ore pulp to beat in air and form a mineral froth in the presence of a small proportion of sodium bisulfate and a small proportion of a mineral frothing agent consisting of a mixture of wood tar oil and Texas fuel oil, separating the froth produced, treating the liquor with free sulfuric acid, and using it with the addition of a further quantity of the mineral frothing agent for the treatment of a further quantity of ore.

In testimony whereof we have signed our names to this specification in the presence of two subscribing witnesses.

GEORGE ALBERT CHAPMAN.  
STANLEY TUCKER.

Witnesses:

ALBERT OWEN WILLIAMS,  
O. J. WORTH.